

# UNITED STATES PATENT OFFICE.

SAMUEL B. CHRONIGER, OF ALLEGHENY, PENNSYLVANIA.

## PLASTIC COMPOUND.

SPECIFICATION forming part of Letters Patent No. 715,022, dated December 2, 1902.

Application filed April 28, 1902. Serial No. 104,990. (No specimens.)

*To all whom it may concern:*

Be it known that I, SAMUEL B. CHRONIGER, a citizen of the United States of America, residing at Allegheny, in the county of Allegheny and State of Pennsylvania, have invented certain new and useful Improvements in Plastic Compounds, of which the following is a specification.

This invention relates to certain new and useful improvements in plastic compounds, relating particularly to such compounds as are employed for wall-plastering and the like; and the object of the invention is to provide a compound extremely cheap to manufacture as well as one embodying advantages over the plaster ordinarily used.

My compound consists of finely-ground natural fire-clay, slaked lime, ground, stucco comprising calcined gypsum rock, ground, dry sand, and goat's hair, which I generally use in about the proportions as follows: finely-ground natural fire-clay, (about) one hundred pounds; stucco, ground, two hundred pounds; slaked lime, ground, twenty-six pounds; dry sand, six hundred pounds; goat's hair, one half pound.

In the manufacture of wall-plaster as here-

tofore used it has generally been the practice to employ quantities of whitening and chalk, which greatly increase the cost of the plaster. 30 By the use of fire-clay in my formula as above given I dispense entirely with whitening and chalk or talc and also lessen the proportion of stucco. In practice I preferably first mix the fire-clay thoroughly with the slaked lime 35 and then add the other ingredients thereto.

It will of course be understood that I do not limit myself to the exact proportions as herein given for the different ingredients, as conditions may require certain alterations in the 40 proportions.

Having fully described my invention, what I claim as new, and desire to secure by Letters Patent, is—

The herein-described compound consisting 45 of finely-ground fire-clay, ground calcined gypsum rock, slaked lime, sand, and goat's hair.

In testimony whereof I affix my signature in the presence of two witnesses.

SAMUEL B. CHRONIGER.

Witnesses:

JOHN NOLAND,  
E. E. POTTER.